

## UNITED STATES PATENT OFFICE

2,108,803

MANUFACTURE AND/OR TREATMENT OF  
ARTIFICIAL MATERIALS

George Holland Ellis and Alexander James Weston, Spondon, near Derby, England, assignors to Celanese Corporation of America, a corporation of Delaware

No Drawing. Application December 29, 1936,  
Serial No. 118,142. In Great Britain January  
16, 1936

9 Claims. (Cl. 8—20)

This invention relates to the saponification of filaments, threads, ribbons, films, fabrics and like materials, having a basis of organic esters of cellulose.

We have found that partial saponification of materials of the kind referred to above in selected areas, renders those areas more sensitive to the action of subsequently applied saponifying agents than are the untreated areas of the material. So marked is this effect that by exposing material which has been locally saponified, to the action of suitable saponifying baths, the saponification in the already saponified areas can be intensified even to the extent of removing substantially the whole of the acidyl content in those areas, without affecting the unsaponified areas. The intensification can be effected by the use of saponifying agents considerably weaker than those employed in the preliminary sensitizing 15 saponification and in fact so weak as not to be regarded normally as saponifying agents at all. The invention provides a method of obtaining intense saponification of local areas only, of materials comprising organic esters of cellulose without undesirable degradation of the cellulose 20 or unevenness of saponification in the selected areas, which therefore dye very evenly.

The preliminary saponification to sensitize the materials for subsequent saponification preferably comprises treatment in the selected areas with an aqueous solution of caustic soda. Other saponifying agents may, however, be used, for example caustic potash or barium hydroxide. The treatment may be a bath treatment applied to materials which have been suitably reserved against saponification in all but the selected areas; or the treatment may be effected by other suitable means, for example by applying the saponifying agent to the selected areas under such conditions that little or no saponification occurs during the actual application and then effecting or completing the preliminary saponification by drying the materials preferably under the influence of heat. Thus, for example, threads or ribbons of cellulose acetate or other organic ester of cellulose may be supplied locally with an aqueous solution of caustic soda and then carried continuously over heated rollers at such a speed that the desired preliminary saponification takes place on the rollers. These may be maintained at a temperature above 100° C. e. g. at 105—110 or 115° C. or at temperatures below 100° C. e. g. 60° C. Instead of heating rollers air drying may be resorted to, the air being maintained e. g., at temperatures between 50 and 110°

C. The temperature at which the saponifying agent is applied, the rate of travel of the materials and the concentration of the saponifying agent may be such that some or even a substantial portion of the preliminary saponification occurs before the materials reach the reaction rollers or drying chamber. The amount of saponification occurring before the rollers are reached may be increased by giving the materials a relatively long air run, e. g., 20—30 feet, between the point of application of the saponifying agent and the rollers. Unduly rapid preliminary saponification is to be avoided and with this in view the lower temperatures specified above are to be preferred. If the sensitized material has any substantial reducing action on Fehling's solution, lower temperatures in the drying chamber or on the reaction rolls and/or lower concentrations of alkali should be tried.

Yarn may also be treated in hank or other suitable package form. Thus for example, hanks or perforated bobbins of the material suitably reserved, may be immersed in a bath containing the saponifying agent under such conditions that the desired preliminary saponification takes place during the time of immersion, or may be immersed without a substantial part or all of the preliminary saponification taking place during application, and may then be dried under the influence of heat or batched at ordinary temperatures, to complete the preliminary saponification step. When the preliminary saponification is effected at relatively low temperatures, e. g., below 50° C., wax-like water-insoluble solid acids such as stearic acid, alone or in admixture with other wax-like substances such as paraffin wax, form the basis of particularly suitable resists as described in U. S. application S. No. 103,204 filed September 29, 1936.

Fabrics may be sensitized locally for subsequent saponification by printing methods or by methods analogous to those described above in relation to the saponification of yarns.

The preliminary saponification may itself be sufficient to impart some affinity for cotton dyes or may be insufficient to affect the dye affinity to any marked extent. Thus the preliminary saponification may remove less than 10% of the original acidyl content of the materials, or from 10 to 15%, or even 20% or more. The smaller the extent of the preliminary saponification, however, the more easily are degradation, unevenness of saponification and other undesirable results avoided. After washing the sensitized materials to remove by-products of the preliminary

saponification, the materials may be dried and collected or may be subjected to the intensification step without drying.

The desired intensification of the saponification in the selected areas may be effected by treatment with an alkaline salt of an alkali metal, for example sodium carbonate, trisodium phosphate, sodium borate, or sodium phenate.

Instead of using alkaline salts non-metallic nitrogenous bases may be used, for example, ammonia and the nitrogenous organic bases. Among nitrogenous organic bases which may be used those in which each carbon atom directly attached to nitrogen is directly attached to three atoms other than the nitrogen are particularly suitable. Examples of such bases are: methylamine, ethylamine, propylamine, butylamine, aminylamine, aliphatic diamines of relatively low molecular weight such as ethylene diamine, symmetrical dimethyl ethylene diamine, amino-ethyl ethylene diamine, and propylene diamine, monoethanolamine, triethanolamine and other alkylamines, cyclic amines such as cyclohexylamine, and benzylamine, in which the amino group is not directly joined to a benzenoid ring, and heterocyclic bases such as piperidine and piperazine. Salts, e. g., sodium acetate, which tend to reduce the swelling action of the organic base on the cellulose ester may be present as described in U. S. Patent No. 2,091,972. The alkaline salt, organic base or other weakly alkaline substance is preferably used in aqueous solution.

The process of the invention is of particular importance in connection with the treatment of materials having a basis of cellulose acetate but is also applicable to the treatment of filaments, threads, yarns, ribbons, films, fabrics and other materials having a basis of other organic esters of cellulose, for example cellulose formate, propionate and butyrate, cellulose acetate-propionate, acetate-butyrate and cellulose laurate and cellulose benzoate. The cellulose ester may be of normal or low viscosity, for example in the case of cellulose acetate the viscosity may be of the order of 30 to 50, 100, 200 or even higher, these figures being obtained by comparison of a 6% solution of the acetate in acetone at 25° C. with glycerine at the same temperature taken as a standard of 100. On the other hand the viscosity of the cellulose acetate may be of the order of 10 to 20 or even lower, or between 20 and 30 measured on the scale referred to above.

The materials may be dyed during or after the saponification. Valuable cross-dye effects may be obtained by locally saponifying the materials to such an extent that the saponified portions acquire an affinity for cotton dyes without losing their affinity for cellulose ester dyes. The saponification may however be such that the affinity for cellulose ester dyes is lost over the saponified parts of the material, and the invention includes complete removal of the acetyl content from the saponified parts of the material.

65 The following examples illustrate the invention:—

#### Example 1

A cellulose acetate yarn is drawn in warp formation, i. e., in the form of a sheet of running yarns, past a device adapted to apply a saponifying agent at intervals along the length of the yarn, through a drying chamber maintained at 50 to 80° C. and through a washing bath to suitable collecting means.

The device for applying the saponifying agent comprises a pair of parallel endless driven chains connected at intervals by transverse slats and dipping at one end of their run, which is inclined, into a trough containing the saponifying agent. Each slat in turn makes contact with the running yarn and transfers to it a quantity of the saponifying agent.

The saponifying agent comprises a 5-6% solution of caustic soda. Other solutions of equivalent alkalinity can be used. The solution is applied at a temperature between 15 and 30° C.

Instead of passing the material through a drying chamber, it may be dried by passage in contact with rolls heated for example by means of hot water.

The treatment renders the portions of the yarn to which the saponifying agent was applied sensitive to further saponification, without affecting the untreated portion.

#### Example 2

Cellulose acetate yarn is drawn in warp formation past a device adapted to apply a resist comprising 85-95% stearic acid and 5-15% paraffin wax, to the yarn at intervals along its length. The device may be of the kind used in Example 1 above for application of the saponifying agent, the trough being filled with the molten resist composition.

The yarn coated with the resist is drawn through an aqueous bath containing 12-15% of caustic soda at a temperature of 30 to 50° C. The speed is adjusted to give a period of immersion of 15 to 30 seconds. Instead of the caustic soda solution other solutions of equivalent alkalinity may be used.

The yarn passes from the saponification bath to a scouring bath in which the resist is removed together with the by-products of saponification.

#### Example 3

Yarn sensitized as described in Example 1 or 2, is immersed in a bath which contains 1 gram per litre of soap and 0.5% caustic soda on the weight of the materials and to which is added gradually in the course of 6 hours a further 5.5% on the weight of the materials of caustic soda. The bath volume is 60:1 and the temperature 60 to 80° C. After immersion for 6 hours the material is removed and is then found to have a good affinity for cotton dyes in the initially sensitized areas and substantially none elsewhere.

#### Example 4

Yarn sensitized as described in Example 1 or 2 is immersed in an aqueous bath of volume about 60 times that of the material and containing 2 grams per litre of soap, 12 to 15% sodium carbonate, 5 to 7½% sodium bicarbonate and 5 to 7½% of sodium acetate, these percentages being based on the weight of the material. The bath is kept at a temperature between 60 and 80° C. and the goods are immersed for ¾ hour to 1 hour. A result similar to that of the preceding example is obtained.

#### Example 5

The process is carried out as in Example 4, except that the bath contains instead of the percentages of alkali metal salts specified, 300% on the weight of the materials of ammonia of specific gravity 0.880 and the time of immersion is extended to 1½ to 2 hours.

## Example 6

5 A shirting cloth containing a mixed warp of ordinary cellulose acetate yarn doubled with a locally saponified cellulose acetate yarn produced as in Example 2 and with a viscose artificial silk 10 yarn and having a weft of ordinary cellulose acetate yarn is immersed in a 2-4% aqueous solution of methylamine. The temperature of the bath is maintained between 15 and 30° C. and 15 the material is immersed therein for from  $\frac{1}{4}$  hour to 1 hour according to the extent of saponification required in the initially sensitized portions of the cellulose acetate yarn.

Very effective cross-dye effects can be obtained 15 by dyeing the so treated fabric with cotton dyes and with dyes for cellulose acetate in succession or in admixture.

## Example 7

20 A fabric of the same structure as that treated in the preceding example is immersed in a bath of volume about 60 times that of the material 25 and containing 1 gram per litre of soap and 62 parts by weight of ethylene diamine per 100 parts by weight of fabric treated. The temperature of the bath is kept at between 75 and 90° C. and the material is immersed for  $\frac{3}{4}$  hour to 1 hour.

## Example 8

30 A cellulose acetate yarn locally sensitized for saponification as described in Example 1 is doubled with an ordinary cellulose acetate yarn and the resulting yarn is used both for the warp 35 and weft of a woven fabric. The fabric is treated in a bath similar to that of the preceding example but with 25 parts of cyclohexylamine on the weight of the goods instead of the ethylene diamine. The time of immersion and temperature are as specified in the preceding example.

40 Fabrics may be sensitized for saponification in the same way as the yarns of Examples 1 and 2 and the saponification intensified as in Examples 3-5. In the sensitization step the presence of a 45 soap in the bath is not essential but is of advantage.

Having described our invention, what we desire to secure by Letters Patent is:—

1. Process for the manufacture of improved 50 artificial textile and like products, which comprises bringing a saponifying agent into contact with selected areas only of threads, fabrics, films or like materials having a basis of organic ester of cellulose, so as to render said areas more 55 sensitive to subsequent saponification, washing the material and thereafter exposing said areas as well as unsaponified areas of the material to a weaker saponifying agent, so as to intensify the saponification of the saponified areas without substantially saponifying the other areas.

60 2. Process for the manufacture of improved artificial textile and like products, which comprises bringing a saponifying agent into contact with selected areas only of threads, fabrics, films and like materials having a basis of cellulose acetate, and thereby effecting a preliminary 65 saponification of said areas so as to render these areas more sensitive to subsequent saponification, washing the materials, and thereafter 70 treating said areas as well as unsaponified areas of the materials with a weaker saponifying agent, so as to intensify the saponification of the saponified areas without substantially saponifying the other areas.

75 3. Process for the manufacture of improved

artificial textile and like products, which comprises bringing a saponifying agent comprising an aqueous solution of caustic soda into contact with selected areas only of threads, fabrics, films and like materials having a basis of cellulose acetate, and thereby effecting a preliminary 5 saponification of said areas so as to render these areas more sensitive to subsequent saponification, washing the materials, and thereafter treating said areas as well as unsaponified areas of the 10 materials with a weaker saponifying agent, so as to intensify the saponification of the saponified areas without substantially saponifying the other areas.

4. Process for the manufacture of improved 15 artificial textile and like products, which comprises applying an aqueous saponifying medium containing caustic soda to selected areas only of threads, fabrics, films and like materials having a basis of cellulose acetate and drying said 20 areas at a temperature above atmospheric, thereby effecting a preliminary saponification of said areas so as to render these areas more sensitive to subsequent saponification, and then washing the materials and thereafter treating said areas 25 as well as unsaponified areas of the materials with a weaker saponifying agent, so as to intensify the saponification of the saponified areas without substantially saponifying the other 30 areas.

5. Process for the manufacture of improved artificial textile and like products, which comprises bringing a saponifying agent comprising an aqueous solution of caustic soda into contact with selected areas only of threads, fabrics, films 35 and like materials having a basis of cellulose acetate, and thereby effecting a preliminary saponification of said areas so as to render these areas more sensitive to subsequent saponification, washing the materials, and thereafter treating 40 said areas as well as unsaponified areas of the materials with a weaker saponifying agent, so as to intensify the saponification of the saponified areas without substantially saponifying the other 45 areas, the preliminary saponification to effect sensitization being carried out by running the material in the direction of its length first past a point at which the saponifying agent is applied to the selected areas, and then through a heated zone where the areas are dried at a 50 temperature above atmospheric and the major part of the preliminary saponification is effected.

6. Process for the manufacture of improved threads, fabrics, films and like materials having a basis of organic ester of cellulose, comprising 55 treating the materials with a saponifying agent after a suitable resist has been applied to parts of the materials which are not to be saponified, thereby effecting a preliminary saponification of the exposed areas so as to render these areas 60 more sensitive to subsequent saponification, washing the materials and removing the resist, and thereafter treating the saponified areas as well as unsaponified areas of the materials with a weaker saponifying agent, so as to intensify 65 the saponification of the saponified areas without substantially saponifying the other areas.

7. Process for the manufacture of improved artificial textile and like products, which comprises bringing an aqueous medium containing 70 a strong mineral alkali into contact with selected areas only of threads, fabrics, films and like materials having a basis of cellulose acetate, and thereby effecting a preliminary saponification of said areas so as to render these areas more sensi- 75

tive to subsequent saponification, washing the materials, and thereafter treating said areas as well as unsaponified areas of the materials with an aqueous solution of an alkali metal salt of 5 alkaline reaction, so as to intensify the saponification of the saponified areas without substantially saponifying the other areas.

8. Process for the manufacture of improved 10 artificial textile and like products, which comprises bringing an aqueous medium containing a strong mineral alkali into contact with selected areas only of threads, fabrics, films and like 15 materials having a basis of cellulose acetate, and thereby effecting a preliminary saponification of said areas so as to render these areas more sensitive to subsequent saponification, washing the materials, and thereafter treating said areas as well as unsaponified areas of the materials with an aqueous solution of ammonia, so as to intensify 20 the saponification of the saponified areas without substantially saponifying the other areas.

9. Process for the manufacture of improved 5 artificial textile and like products, which comprises bringing an aqueous medium containing a strong mineral alkali into contact with selected areas only of threads, fabrics, films and like 10 materials having a basis of cellulose acetate, and thereby effecting a preliminary saponification of said areas so as to render these areas more sensitive to subsequent saponification, washing the materials, and thereafter treating said areas as 15 well as unsaponified areas of the materials with an aqueous solution of an organic nitrogenous base in which each carbon atom directly attached to nitrogen is also directly attached to three other atoms, so as to intensify the saponification 20 of the saponified areas without substantially saponifying the other areas.

GEORGE HOLLAND ELLIS.  
ALEXANDER JAMES WESSON. 20